

## UNITED STATES PATENT OFFICE.

HERBERT THEODORE PRICE, OF BURWOOD, SYDNEY, NEW SOUTH WALES, AUSTRALIA.

## PULP BOARD AND PROCESS OF MANUFACTURING THE SAME.

No Drawing. Application filed April 13, 1927, Serial No. 183,626, and in Australia June 14, 1926.

This invention is for an improved pulp board and process of manufacturing the same.

It is known that megass, a fibrous by-product in the manufacture of sugar, has valuable properties as a pulp for board making, and is applied to that purpose with success. Board, however, made from megass alone is rather brittle when rolled into thin sheets, and thickness increases the cost and weight, and such sheets are more difficult to dry.

The object of my invention is to provide an improved pulp board in which megass is a largely constituent part, and which will be tougher and lighter, and capable of thin rolling or pressing, at the same time having a fine surface. My invention also provides a process of manufacturing the improved pulp board.

20 A pulp board made according to this invention consists essentially of megass and ti-tree or bark of the ti-tree or both commonly found on swampy land. I have found that the addition of ti-tree or bark effects a more rapid drying of the finished board.

25 My process consists in first soaking the megass in a solution of caustic soda to soften and clean it. After soaking, the megass is mixed with finely ground ti-tree and/or bark of the ti-tree.

30 I have found that good results are obtained by a mixture of eighty per cent by weight of the megass and twenty per cent of the ti-tree bark although other proportions give satisfactory results.

35 After the mixing, the pulp is of good consistency and is taken away by conveyors to be boiled in a solution of caustic soda or lime. This boiling is under steam and takes one to two hours.

40 After cooking, the pulp is conveyed on a woven wire belt, and above this belt is another woven wire belt adapted to be lowered on to the pulp held in the belt beneath. The belts are so mounted that they have a short and sharp to and fro motion in opposite directions to each other and the upper belt also has a short and rapid up and down motion relative to the lower belt. This motion forces the fibrous parts of the megass to the bottom of the intended board and brings the lighter substance such as ti-tree bark and pith of the megass to the surface.

The board is finished off in the usual board

forming manner and is useful for numerous purposes.

I claim:

1. An improved pulp board comprising finely ground ti-tree.

2. An improved pulp board comprising finely ground ti-tree bark.

3. An improved pulp board comprising finely ground ti-tree and ti-tree bark.

4. An improved pulp board comprising megass; and finely ground ti-tree.

5. An improved pulp board comprising megass; and finely ground ti-tree bark.

6. An improved pulp board comprising megass; and finely ground ti-tree and ti-tree bark.

7. An improved pulp board comprising approximately 80 per cent of megass and twenty per cent of finely ground ti-tree.

8. An improved pulp board comprising approximately 80 per cent of megass and twenty per cent of finely ground ti-tree bark.

9. An improved pulp board comprising approximately 80 per cent of megass and twenty per cent of finely ground ti-tree and ti-tree bark.

10. In a method of manufacturing pulp board comprising the steps of soaking megass in a caustic soda solution, mixing the megass with ti-tree, grinding the megass and ti-tree, and boiling the mixed megass and ti-tree in a caustic soda solution.

11. In a method of manufacturing pulp board comprising the steps of soaking megass in a caustic soda solution, mixing the megass with ti-tree, grinding the megass and ti-tree, and boiling the mixed megass and ti-tree in a lime solution.

12. In a method of manufacturing pulp board comprising the steps of soaking megass in a caustic soda solution, mixing the megass with ti-tree bark, grinding the megass and ti-tree bark, and boiling the mixed megass and ti-tree bark in a caustic soda solution.

13. In a method of manufacturing pulp board comprising the steps of soaking megass in a caustic soda solution, mixing the megass with ti-tree and ti-tree bark, grinding the megass and ti-tree and ti-tree bark, and boiling the mixed megass and ti-tree and ti-tree bark in a caustic soda solution.

14. In a method of manufacturing pulp board comprising the steps of soaking megass in a weak solution of caustic soda, mixing ap-

proximately 80 percent of the megass with 20 percent of ground ti-tree, grinding the megass and tie-tree, and boiling the ground megass and ti-tree in a weak caustic soda solution for several hours.

15. In a method of manufacturing pulp board comprising the steps of soaking megass in a weak solution of caustic soda, mixing approximately 80 percent of the megass with 20 percent of ground ti-tree bark, grinding the megass and ti-tree bark, and boiling the ground megass and ti-tree bark in a weak caustic soda solution for several hours.

16. In a method of manufacturing pulp board comprising the steps of soaking megass in a weak solution of caustic soda, mixing approximately 80 percent of the megass with 20 percent of ground ti-tree and ti-tree bark, grinding the megass and ti-tree and ti-tree bark, and boiling the ground megass and ti-tree and ti-tree bark in a weak caustic soda solution for several hours.

17. In a method of manufacturing pulp board comprising in conveying the pulp to the presses between parallel woven wire belts, and rapidly moving the belts in intermittent to and fro motions in opposite directions to each other and moving one belt away from and toward the other belt to provide a readjustment of the substances in the pulp.

18. In a method of manufacturing pulp board comprising in conveying the pulp between parallel wire belts, and rapidly moving the belts in intermittent to and fro motions in opposite directions to each other and moving the upper belt rapidly away from and toward the lower belt to provide a readjustment of the substances in the pulp.

19. In a method of manufacturing pulp board comprising in conveying the pulp be-

tween two parallel foraminiferous belts, and moving the belts in intermittent to and fro motions in opposite directions to each other and at the same time moving the upper belt rapidly away from and toward the lower belt 45 to work the long and coarse fibres of the pulp to the bottom and the fine fibres to the top and the intermediate fibres in regular graduation therebetween.

20. In a method of manufacturing pulp board comprising in arranging the fibres of the pulp so that the long and coarse fibres will be at the bottom and the fine fibres at the top, and the intermediate fibres in regular graduation therebetween. 50

21. In a method of manufacturing pulp board comprising conveying the pulp between two parallel foraminiferous belts moving in short and rapid reciprocating motions in opposite directions to each other and also one 55 belt rapidly up and down relative to the other belt to arrange the fibres of the pulp.

22. In a method of manufacturing pulp board comprising conveying the pulp between two parallel foraminiferous belts moving in short and rapid reciprocating motions in opposite directions to each other and the upper belt having a short up and down motion relative to the lower belt to arrange the fibres 60 of the pulp. 65

23. In a method of manufacturing pulp board comprising conveying the pulp between two parallel foraminiferous belts the upper of which has a short rapid up and down motion relative to the lower belt to arrange the 70 fibres of the pulp. 75

In testimony whereof I have affixed my signature.

HERBERT THEODORE PRICE.